

# United States Patent [19]

Kamigaito et al.

[11] 3,967,230

[45] June 29, 1976

[54] RESISTOR BUILT-IN SPARK PLUG

[75] Inventors: Osami Kamigaito; Haruo Doi; Hideyuki Masaki; Toshio Kandori; Masami Oki; Yasuo Nakamura, all of Nagoya, Japan

[73] Assignees: Nippondenso Co., Ltd.; Kabushiki Kaisha Toyota Chuo Kenkyusho, both of Japan

[22] Filed: Oct. 22, 1974

[21] Appl. No.: 517,053

[30] Foreign Application Priority Data

Nov. 12, 1973 Japan ..... 48-127032

[52] U.S. Cl. ..... 338/66; 123/148 P; 123/169 R

[51] Int. Cl.<sup>2</sup> ..... H01C 1/06; H01C 7/06

[58] Field of Search ..... 338/66; 123/148 P, 169 R, 123/148 R; 29/25.12

[56] References Cited

UNITED STATES PATENTS

2,371,211 3/1945 Barrington ..... 338/66

2,436,644 2/1948 Halstead ..... 338/66

Primary Examiner—C. L. Albritton  
Attorney, Agent, or Firm—Cushman, Darby & Cushman

[57]

## ABSTRACT

A resistor built-in spark plug comprises an insulator formed with an axially extending inner hole, a stem fitted in the upper part of said hole in said insulator, a center electrode fitted in the lower part of said hole, a resistor disposed in the central part of said hole, and copper-glass electrode layers disposed between said resistor and said stem and between said resistor and said center electrode. Said resistor is made by firing and solidifying powder of resistor mixture consisting of 75 to 38 volume percent of main resistor component containing tin oxide and 25 to 62 volume percent of glass powder with softening temperature of 300° to 600°C. Said copper-glass electrode layers are made by firing and solidifying a mixture of copper powder and glass powder with the softening temperature of above 530°C and more than 30°C higher than the softening point of glass in the resistor portion.

12 Claims, 3 Drawing Figures



FIG. 3



FIG. 2



FIG. 1



## RESISTOR BUILT-IN SPARK PLUG

This invention relates to the improvements in the resistor built-in spark plugs which have noise suppressing effect for the radio wave.

Necessity has been voiced for preventing noise of the communication radio waves by the electric waves produced by the spark plugs. As a measure for preventing such noise, it has been proposed and already commonly practiced to incorporate a resistor in the electric circuit of a spark plug. There are known two methods of incorporating a resistor: setting it in a hole formed in an insulator of the spark plug or setting it in a high-tension wire in the ignition circuit.

The resistivities of the resistors usable for prevention of noise of the radio waves are regulated under the JIS rules into the following three ranges:  $5 \text{ K}\Omega \pm 30\%$ ,  $10 \text{ K}\Omega \pm 30\%$  and  $15 \text{ K}\Omega \pm 30\%$ . As regards the properties of the resistors, the rate of change of resistivity after the spark discharge test and the heating test is also regulated. That is, it is ruled that the change of resistivity after 250 hours of spark discharge must be less than  $\pm 25\%$  and  $-40\%$  of the respective resistivities in said three defined ranges, and that the change of resistivity after heating to  $350^\circ\text{C}$  and then cooling must be less than  $\pm 25\%$  of said resistivities.

There have heretofore been proposed various types of resistors which meet the above-said standard requirements, but most of such resistors have been prepared by shaping and solidifying an electroconductive material with glass for easy incorporation in spark plugs. As such electroconductive material, or the main component of the resistor, is generally used powder of metal (such as copper, iron, nickel, or nickel-chromium alloy) or carbon, or powder of low-resistance metal oxides (such as zinc oxide, barium oxide or nickel oxide). However, the resistors manufactured from such material and glass are low in specific resistance, usually less specimen  $0.01 \Omega\text{-cm}$ , and the resistors with such low specific resistance show almost no noise suppressing effect because the resistance thereof becomes small value of less than  $0.1 \Omega$ . Resistivity of such resistors can be elevated by increasing the amount of glass added, but this means, on the other hand, that such resistivity is subjected to wide change according to increase or decrease of the amount of glass added. Thus, such resistors didn't suit the practical use.

The present inventors have entertained the idea of using the resistant material mainly composed of tin oxide, described in our previous applications Pat. Nos. 47-95439, 47-109724 and 47-112363, as the main component material of resistor used in the spark plugs of the present invention. The resistors obtained by using such component material including tin oxide provide a resistivity of several  $\text{K}\Omega$  to several ten  $\text{K}\Omega$ , which is the level required for practical applications. Further, such value of resistivity is not widely changed according to the amount of glass added in the main component material including tin oxide.

There was however found out a new problem that the resistivity of the resistor varies depending on the properties of glass blended in the main component material including tin oxide. This problem is not limited to the material including tin oxide but applies similarly to other materials which have heretofore been used as main components. That is, in case of using glass same as that in the copper-glass layer (mixture of copper

powder and glass powder) in the electrode popularly used in manufacture of spark plugs, or in case of using glass which has no much difference in properties from or somewhat worth in fluidity than glass in said copper-glass layer, the interface of said copper-glass layer and the resistor is curved parabolically and the resistivities of the obtained resistors vary widely from one another, so that it is hardly possible to obtain the resistor built-in spark plugs with uniform resistivity.

10 The present inventors have found as a result of numerous tests and experiments that such curving of the interface is ascribed to the difference in the degree of local softening and fluidity between glass in said copper-glass layer in the electrode and glass in the resistor.

15 In view of the above, the present invention proposes a method of obtaining the improved and very useful resistor built-in spark plugs with limited variations in resistivity, according to which method a resistor mixture consisting of powder of the main component material

20 including tin oxide and glass powder with softening temperature of  $300^\circ$  to  $600^\circ\text{C}$  and in an amount of 25 to 62 volume percent of said main component material is placed in a hole formed in an insulator, then a copper-glass layer (for electrode) formed from a mixture

25 of copper powder and glass powder with softening temperature of above  $530^\circ\text{C}$  and more than  $30^\circ\text{C}$  higher than that of glass in the resistor portion is disposed between said resistor mixture and a middle stem fitted in one part of an inner hole formed in said insulator and between said resistor mixture and the center electrode fixed in said hole on its side opposite from said stem, and then all of these materials are fired so that they are solidified integral with each other.

30 In the present invention, as a powder mixture containing tin oxide is used as the main component of the resistor, it is possible to obtain a resistor built-in spark plug having resistivity of from  $3.5$  to  $19.5 \text{ K}\Omega$  which is the level required for effective prevention of noise of radio waves. Particularly, in the present invention, glass

35 with softening temperature of from  $300^\circ$  to  $600^\circ\text{C}$  is used as glass added to the powder mixture containing tin oxide, and such glass is blended in an amount of 25 to 62 volume percent to said powder mixture. Also, glass in the copper-glass layers between the powder mixture and middle stem and between said powder mixture and center electrode is of the type that has softening temperature of higher than  $530^\circ\text{C}$ . Further, in case the softening temperature of glass in the resistor

40 portion is in the range of  $500^\circ$  to  $600^\circ\text{C}$ , glass with softening temperature more than  $30^\circ\text{C}$  higher than that of glass in said resistor portion is used as glass in the copper-glass layers. There are therefore obtained the very excellent resistor built-in spark plugs with extremely limited variations of resistivity. The resistivity

45 after the spark discharge test, heating test and engine endurance test is not much different from that before such tests.

The main resistor mixture according to the present invention contains, besides tin oxide, one or more of 50 the following materials: carbon powder, metal oxide metal, antimony oxide, aluminium phosphate, organic binder, and filler.

55 The reasons for defining the amount of glass powder to be blended in the main resistor mixture, the softening temperature of such glass powder and the softening temperature of glass in the copper-glass layers of electrode will become apparent from the following description.

The present inventors gave particular attention to the causes of curving of the aforementioned interfacial boundary and have found that such curving can be avoided by eliminating the difference in the degree local softening and fluidity between glass in the copper-glass layers and glass in the resistor. For uniformizing such local softening and flow of glass, there seems available no other way but to either make the resistor itself into a substantially solidified mass or to turn it into a liquid state so that wall surface resistance and flow resistance in the hole in the insulator will become negligibly low as compared with resistance of the copper-glass layers positioned above and below the resistor. The present inventors have first studied the latter method for some reasons combined. In order to give sufficient fluidity to the resistor or filler, it needs to make fluidity of glass used therein better than that of glass used in the copper-glass layers positioned above and below said resistor. Therefore, the kind and composition of glass used in the resistor may vary widely depending on the properties of glass used in the copper-glass layers or the amount of copper powder blended in said layers. However, since the filler, or resistor, and the copper-glass layers of the electrode must be hermetically sealed in the hole formed in the insulator and also the spark plug is exposed to high temperatures in use, either of the glass materials used must have sufficient strength to withstand such high temperatures. As already mentioned, in order to make fluidity of glass blended in the resistor portion sufficiently higher (at same temperature) than fluidity of glass blended in the copper-glass layers, it is essential that glass used in the copper-glass layers has a softening point higher than a certain level. Such softening point must be also lower than a certain value, because if the softening point is too high, it becomes impossible to use inexpensive steel material for the middle stem and center electrode.

With these facts in mind, the present inventors have reached the conclusion that glass used in the copper-glass layers should be the type having the softening point of higher than 530°C but preferably not higher than 750°C, such as for example soda-lime glass. If pulverized copper is mixed in glass having the softening point of said range, the softening point of the entire mixture becomes about 20° to 50°C higher than that of glass not yet mixed with pulverized copper. It is essential therefore that the softening point of glass in the resistor is lower than 750°C. As the spark plug is raised in temperature to about 250°C during use, glass in the resistor should obviously have a softening point of higher than 250°C. The above-said range (250° to 750°C) of the softening point of resistor glass shows the values required in principle. Therefore, the actual upper and lower threshold limit temperature are experimentally determined by taking into consideration the amount of glass blended, as further discussed below.

The invention will be further described with reference to the accompanying drawings in which:

FIG. 1 is a longitudinal sectional view of the resistor built-in spark plug according to the first embodiment of the invention;

FIG. 2 is a longitudinal sectional view of the resistor built-in spark plug according to the second embodiment of the invention; and

FIG. 3 is a longitudinal sectional view of the resistor built-in spark plug according to the third embodiment of the invention.

The amount of glass to be blended in the main component mixture of the resistor varies depending on whether the resistor is sealedly contained in the spark plug or whether it is placed in solid form in said plug. In the present invention, as the former method is employed as shown in FIGS. 1, 2 and 3, the amount of such blended glass must be sufficient to allow the fine particles themselves of the resistor mixture to adhere strongly to each other and also the resistor 3 thereof to bond to the upper and lower copper-glass layers 4, 5 as well as to the interior surface of the inner hole 1a in the insulator 1. The results of experiments conducted by the present inventors showed that the amount of glass required therefor is 25 to 62 volume percent of the main component mixture.

If the amount of glass blended in the resistor 3 is smaller than 25 volume percent of the component mixture, the resistivity of the obtained resistor built-in spark plugs tends to vary widely after the spark discharge test, engine endurance test and heating test (see Table 2). This is probably because certain movement, fall-off and separation or adhesion take place in the main component mixture due to expansion or contraction caused by temperature change as the glass amount is too small.

It was also found that if the amount of glass blended in the component mixture exceeds 62 volume percent of said mixture, the resistivity of the obtained spark plugs varies widely between the individual plugs, and such resistivity could be also sharply lowered or elevated by the spark discharge (see Table 2). This is considered attributable to the fact that if the amount of glass blended exceeds 62 volume percent, a thick glass film is formed between the adjoining particles of the mixture powder to prevent contact between such individual particles, and this probably causes wide variations of resistivity in some cases. It is also considered that when spark discharge is performed, said glass film is broken with flow of current to the spark plug to cause decrease of resistivity, or the relatively thin glass film broken by current flow is melted to cause leakage in the contact portions of the resistor 3 and the copper-glass layers 4, 5 to induce elevation of resistivity.

In either case, the results of our experiments show that the amount of glass to be blended in the component mixture should preferably be within the range of 25 to 62 volume percent of the component mixture no matter what kind of glass is used.

It was also confirmed as a result of numerous experiments that when the amount of glass blended in the component mixture is selected from the above-defined range, the softening point of such glass should preferably be lower than 600°C, although there is actually a lower threshold limit value for such softening point. As aforesaid, the spark plug itself is heated to a high temperature of about 250°C in use, so that when using glass with softening point of around 250°C, the resistor 3 in the insulator is softened to inevitably induce variations in resistivity. Therefore, the lower threshold limit value of softening point of glass used in the resistor 3 is theoretically 250°C, but it actually needs to give a certain safety allowance and hence such lower threshold limit value should, in practice, be 300°C. It was also observed that if the softening temperature of glass used in the resistor exceeds 620°C, no satisfactory fusion-bonding between the resistor portion and insulator can be accomplished by a hot press of the type used in a temperature range safe from causing oxidation of the

stem and center electrode, resulting in excessive variation of resistivity by heating. Further, since the softening point of glass in the copper-glass layers is higher than 530°C, if glass with softening point of higher than 530°C is used for the resistor portion, it could happen that the softening point of glass in the copper-glass layer becomes higher than that of glass in the resistor portion. In such cases, variations in resistivity are widened almost without exception, and the yield of the spark plugs that meet the  $5 \text{ K}\Omega \pm 30$  percent range requirement is markedly lowered. It has however admitted that such variations in resistivity can be minimized if suitable glass combination is selected such that the softening point of glass in the copper-glass layers will be more than 30°C higher than that of glass in resistor portion. It was thus found necessary for obtaining excellent spark plugs to select such kind of glass for resistor portion as having the softening point within the range of 300° to 600°C and such kind of glass for the copper-glass layers that its softening point will be more than 30°C higher than that of resistor glass when the softening point exceeds 500°C. In case the softening point of glass in the copper-glass layer is not higher than that of resistor glass by more than 30°C when the softening point of the resistor glass is 500° to 600°C, there was observed a tendency that the interfacial boundaries of the resistor portion and the copper-glass layers are curved, and this is considered responsible for wide variations in resistivity. Such curving of the interfacial boundaries is considered attributable to the fact that fluidity of the copper-glass layers becomes substantially equal to that of the resistor portion to give rise to a flow such as above-said.

The present inventors have also found that if the coefficient of thermal expansion of glass in the resistor 3 and in the copper-glass layers 4, 5 is as high as over  $11.3 \times 10^{-6}/^\circ\text{C}$ , cracks could develop in said resistor portion 3 or in the copper-glass layer portions 4, 5, resulting in a spark plug with extremely high resistivity. This is probably due to shrinkage that was caused in the cooling step after manufacture of the spark plug. It was found that development of such cracks could be controlled to some extent by using a filler with low swelling characteristic. It is however preferable, generally, to use glass with coefficient of thermal expansion of less than  $11.3 \times 10^{-6}/^\circ\text{C}$ . The term "filler" as used here refers to a material (pulverized) having extremely high electric resistivity, such as for example quartz glass, zirconia and zircon. On the other hand, if the coefficient of thermal expansion of glass is too low, strain may be produced in the insulator 1 during the cooling step after manufacture of the spark plug, and such strain may develop cracks in the insulator 1. However, coefficient of thermal expansion of glass is usually not so low, so that, actually, there is little possibility of obtaining and using glass with such low coefficient of thermal expansion as could cause cracks. No crack developed in the low-expansibility glass ( $\alpha = 4.3 \times 10^{-6}/^\circ\text{C}$ ) that the present inventors could obtain, so if judging merely from the aspect of cracking, it is possible to use glass with coefficient of thermal expansion ( $\alpha$ ) of up to  $4.3 \times 10^{-6}/^\circ\text{C}$ . Further, if a high expansibility material is used as filler, since high expansibility is maintained during the cooling step of the obtained spark plug, shrinkage is promoted to form pores in the resistor portion and such pores prove helpful to lessen thermal stress. Also, greater strength can be assured by increasing the glass thickness. Thus, substantially no particular restriction

is imposed by the low coefficient of thermal expansion of glass used.

Referring here to the drawings, FIG. 1 shows the construction of a resistor built-in spark plug in which the copper-glass layers 4, 5 of the electrode are disposed one above and the other below the resistor 3. In study of this construction, the present inventors have found that if the copper-glass layer 4 positioned above the resistor 3 is divided into two layers 4a and 4b as shown in FIG. 2 and if the first layer 4a contacted with the resistor 3 is blended with greater amount of copper than that blended in the second layer 4b which is in contact with the middle stem 2, the variations in resistivity of the obtained resistor built-in spark plugs are significantly limited as compared with those observed when using high expansibility glass in the resistor of the spark plug with the construction of FIG. 1 even if coefficient of expansion of glass in the resistor 3 is high (see Tables 2 and 4). It was also found as a result of numerous experiments by the present inventors that if the copper-glass layers and resistor 3 in the hole 1a in the insulator 1 are arranged in five layers as shown in FIG. 3, that is, if each of the copper-glass layers on both upper and lower sides of the resistor 3 is bisected to form the first, second, third and fourth copper-glass layers 4a, 4b, 5a and 5b, and if the first and third layers 4a and 5a in contact with the resistor 3 are blended with a greater amount of copper than that blended in the second and fourth layers 4b and 5b which are contacted with the stem 2 and the center electrode 6, respectively, the variations in resistivity can be even more diminished. The above-described results can be obtained by using lead borate glass, zinc borate glass, lead glass, zinc-soda glass or the like as glass in the resistor 3 in the resistor built-in spark plug of the construction shown in FIG. 2 or FIG. 3.

The present invention is now described in further detail by way of some preferred embodiments thereof, but these embodiments are by no means restrictive but merely illustrative of the present invention.

#### FIRST EMBODIMENT

There were prepared various types of glass powder specimens (No. 1 to No. 22) (all passing 200-mesh screen) as shown in Table 1. There was also prepared powder of main component mixture of resistor (hereinafter referred to as main resistor mixture) containing tin oxide added with 3 wt percent of antimony oxide and 10 wt percent of tantalum oxide, then burned at 1200°C and then pulverized. A suitably measured amount of each of said various types of glass powders and said main resistor mixture were collected and then mixed well in a ball mill. There was further prepared mixture powder comprising 50 wt percent of copper powder (all passing 200-mesh screen) and 50 wt percent of each of glass specimens shown in Table 1 (such mixture being hereinafter referred to as 50-copper-glass mixture).

In the meanwhile, there were also prepared alumina-made insulators 1 (inner diameter  $4.8 \text{ mm}$ ), center electrodes 6 and middle stems 2 such as shown in FIG. 1. First, a center electrode 6 was inserted bottomwise into an inner hole 1a in the insulator 1, and then about 0.2 gr of 50-copper-glass mixture powder was charged into said hole 1a in the insulator 1 and a pressure of about 50 kg/cm<sup>2</sup> was applied to said 50-copper-glass mixture by using a press to flatten the top surface of the mixture. Then about 0.5 gr of mixture of said main resistor

mixture powder and glass powder was poured onto said copper-glass layer and again a pressure was applied thereto to flatten the top surface thereof. Then, again, about 0.3 gr of 50-copper-glass mixture powder was charged onto said mixture, followed by topwise insertion of a stem 2 into said hole 1a and application of pressure to said stem 2. Thereafter, the insulator 1 was placed in a furnace which consists of an electric heater of silicon monoxide (so-called siliconit) and is maintained at high temperature of 890°C, and after left therein for about 30 minutes, said insulator was taken out and a pressure of about 200 kg was applied to the stem 2 by a press to effect bonding and compression of the particles loaded in the inside of the insulator. This final operation turned the 50-copper-glass mixture on the center electrode 6 into a copper-glass layer 5, the mixture of main resistor mixture powder and glass powder into a resistor 3, and the 50-copper-glass mixture contacting the stem 2 into a copper-glass layer 4 of the electrode. After cooling the insulator 1, a housing 7 was mounted around said insulator to obtain a resistor built-in spark plug.

100 pieces of spark plugs were manufactured by following the same process as described above for each of the glass specimens (No. 1 to No. 22) of Table 1, and the following matters were examined over each 100-piece group of the obtained spark plugs: per cent defectives (or the rate of the articles whose average resistivity and JIS regulated resistivity were outside the range of  $5 \text{ K}\Omega \pm 30$  percent), increase (in percentage) of the average resistivity after 1-minute spark discharge over the average resistivity before the test, increase (in percent) of the average resistivity after 1-minute spark discharge test, heating to 250°C and then cooling over the average resistivity before the test, and increase (in percent) of the average resistivity after engine endurance test (conducted by attaching the device directly to the engine) over the average resistivity before the test. The results are shown in Tables 2-1 to 2-3. The substantial length of the resistor 3 in each of the spark plugs obtained by the above-said method is approximately 7 mm if the interfacial boundaries of the resistor 3 and the copper-glass layers 4, 5 of the electrode are flat. As apparent from Tables 2-1 to 2-3, if the amount of glass blended is greater than 62 volume percent of the main resistor mixture, the resistivities of the obtained spark plugs vary widely from plug to plug and such resistivities are also greatly changed by the spark discharge test, irrespective of the composition of glass used in manufacture of the resistor 3. To be more concrete, if No. 5 specimen of Table 1 is used as glass for the resistor 3 and this glass is blended in an amount of 63 volume percent of the main resistor mixture, the defectives (or the articles whose resistivity is outside of the range of  $5 \text{ K}\Omega \pm 30$  percent, one of the resistivity ranges regulated by JIS) accounts for 63 percent of the entire products. This means that 63 out of every 100 articles obtained are defective. It will be understood from this fact that the resistivities of the obtained products vary so widely from product to product. It is to be also noted that the average resistivity after one-minute spark discharge test shows an 8 percent increase over the average resistivity before the test, while that after the engine endurance test shows a 10 percent increase. On the other hand, if the amount of glass blended is smaller than 25 volume percent of the main resistor mixture, there is also observed a tendency that the resistivities of the obtained spark plugs vary widely

5 from plug to plug and such resistivity also undergoes wide variation after the heating test conducted by heating each article to 250°C after one-minute spark discharge test. To put it more concretely, if glass of specimen No. 5 in table 1 is used as glass component of the resistor and this glass is blended in an amount of 20 volume percent of the main resistor mixture, the obtained spark plugs with resistivities outside the range of  $5 \text{ K}\Omega \pm 30$  percent accounts for 80 percent of the entire products, which shows how wide are the variations in resistivities of the obtained articles. Also, the average resistivity after the heating test shows as much as 25 percent increase over the average resistivity before the test. These results dictate that the amount of glass used in the resistor should preferably be within the range of 25 to 62 volume percent of the main resistor mixture. However, even if glass is used in an amount within said range, although the resistivity variation after the spark discharge test, heating test and engine endurance test is significantly limited, it is noted (as apparent from Tables 2-1 to 2-3) that the resistivities of the individual spark plugs still differ widely from one another, notwithstanding the fact that the amount of glass blended is within the above-said range (25 to 62 volume percent). This is indicative of the fact that the softening point of glass used in the resistor exerts as great influence to the spark plug resistivity as the amount of glass blended.

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 1

glass in the resistor portion differs by less than 10°C from that of glass in the copper-glass layers, or the former is higher than the latter. In these combinations, it is considered that bad flow in the resistor portion is responsible for the above-said results as expected at the beginning. On the other hand, even when using glass of specimen Nos. 1, 2, 9, 12, 17 and 21, if the softening point of glass in the copper-glass layers is higher by more than 30°C than that of glass in the resistor portion, excellent results are obtained, or at least better results are obtained than when using glass with smaller temperature difference. Interior examination of these spark plugs revealed flat interfacial boundaries indicative of excellent properties of the products. These results show that the softening point of glass used in the resistor portion should be lower by more than 30°C than that of glass used in the copper-glass layers. It is also noted from Table 2-1 that if glass of specimen No. 4 is blended in the main resistor mixture in an amount of 50 volume percent of said mixture, the average resistivity after the engine endurance test shows an increase of 20 percent of the average resistivity (5.8 KΩ) before the test, and also change of resistivity after the spark discharge test and the heating test is very limited. The softening point of glass of No. 4 is 360°C. Although not shown in Table 2, the results of experiments by the present inventors have also revealed that the variations in resistivities and change of resistivity after each test are limited within a very small scope even if the softening point of glass used is 300°C. The reason for defining the softening point to not lower than 300°C will be evident from the foregoing description, too. Anyway, the most preferred range of softening point of glass used in the resistor is from 300° to 600°C. Thus, it is preferred that the amount of glass used in the resistor is within the range of 25 to 62 volume percent of the main resistor mixture and that the softening point of glass used therefor is within the range of 300° to 600°C. It is also desirable that softening point of glass used in the copper-glass layers of electrode is higher than 530°C and that when using glass with softening point of higher than 500°C for the resistor portion, glass used in the copper-glass layers has the softening point 30°C higher than that of glass used in the resistor portion. It is also noted from Tables 2-1 and 2-2 that when using glass with coefficient of thermal expansion of greater than  $11.3 \times 10^{-6}/^{\circ}\text{C}$  for the resistor, there are observed certain cases where the degree of scatter of resistivities or fraction defective is high although the glass used meets the above-said definitions, but generally, the scatter of resistivities is limited and good results are obtained if the above-said definitions are met. Even when glass with thermal expansion coefficient of greater than  $11.3 \times 10^{-6}/^{\circ}\text{C}$  is used for the resistor under the above-said conditions, it is possible to reduce the scatter of resistivities to certain extent as discussed in the following second and third embodiments which are modifications of the foregoing first embodiment of the invention. As viewed above, there are provided according to the present invention the excellent resistor built-in spark plugs which are generally low in the scatter of resistivities and in which change of resistivity after the spark discharge test and heating test is less than 10 percent and that after the engine endurance test is less than 8 percent.

Now, a modification of the above-described first embodiment of the present invention is described.

As shown in Table 3, there were prepared quartz glass powder (all passing 200-mesh screen), zirconia powder (all passing 200-mesh screen) and zircon powder (all passing 200-mesh screen) as filler, and the main resistor mixture powder (all passing 200-mesh screen) containing tin oxide ( $\text{SnO}_2$ ) added with 3 wt percent of  $\text{Sb}_2\text{O}_3$  and 3 wt percent of  $\text{Ta}_2\text{O}_5$ . There were also prepared powders (all passing 200-mesh screen) of glass of specimen Nos. 1, 3, 4, 5, 8, 12, 14 and 20 in Table 1. Then these powders were mixed in suitable amounts and combinations and the resistor built-in spark plugs were manufactured by following the same steps as the first embodiment. The resistivities of these spark plugs and the results of tests conducted on these plugs after the fashion of the first embodiment are also shown in Table 3. As seen in the same table, if the amount of glass used is within the range of 25 to 62 volume percent of the mixture of tin oxide-containing main resistor mixture and filler and the softening point of such glass is less than 600°C, variations in resistivities of the obtained spark plugs are limited and also change of resistivity after the spark test, heating test and engine endurance test is very small as in the case of the first embodiment. If a low-expansibility filler (such as quartz glass) is used, the fraction defectives, or the rate of articles whose resistivities are outside the range of  $5 \text{ K}\Omega \pm 30\%$  (3.5 – 6.5 KΩ) is 20 percent, that is to say, the number of defective articles is 20 out of every 100 articles produced, even when using glass with high expansion coefficient such as glass of specimen No. 14 ( $\alpha = 14.0 \times 10^{-6}/^{\circ}\text{C}$ ). This is a marked improvement over 45 percent defective rate of the articles using glass of specimen No. 14 in Table 2-1. The same is true of glass of specimen No. 20 if such glass is used in an amount of 41 volume percent of the main resistor mixture containing tin oxide. Thus, high coefficient of thermal expansion of glass used in the resistor is not an inherent defect, and it is apparent that such problem can be avoided by employing a suitable means, for example by use of a filler. Therefore, the fact that use of filler can minimize variations in resistivities implies that resistivity of the resistor can be changed by use of a filler. In other words, this effect of the filler is suggestive of the fact that if a same resistor is prepared, it is possible to obtain a resistor built-in spark plug having a desired resistivity by using a filler. It will be thus understood that use of a filler is of great significance in practical use.

The number of experiments conducted in connection with this modification of the first embodiment is small as compared with that in the first embodiment, but this is due to the fact that the present inventors have practiced this modification on the basis of the first embodiment. Therefore, the softening temperature of glass to be added in the main resistor mixture (containing tin oxide), the amount of glass to be added, and the softening temperature of glass used in the copper-glass layers of electrode are of course same as those in the first embodiment.

Now, the second and third embodiments of the present invention are described. In the second embodiment, there were prepared glass powders (wholly passing 200-mesh screen) of specimen Nos. 4, 5, 9 and 14 in Table 1 as well as a main resistor mixture containing tin oxide added with 3 wt percent of antimony oxide and 10 wt percent of tantalum oxide, then burned at 1200°C and then pulverized. Thereafter, each of said glass specimens and the main resistor mixture were

collected in suitable measured amounts and mixed well in a ball mill. There were also prepared copper powder (all passing 200-mesh screen) and glass of specimen Nos. 1 to 3 of Table 1, and both were mixed at the respectively predetermined rates to obtain mixture powders. Then the mixture of said copper powder and glass and was first charged onto the center electrode 6 in the hole 1a in the insulator 1 and then the mixture of tin oxide-containing main resistor mixture and glass was charged thereon, followed by additional charging thereon of a mixture same in composition as but different in amount of copper powder added from said mixture and further application thereon of said mixture. Thereafter, the middle stem 2 was inserted topwide into the hole 1a and then subjected to hot press, thereby forming said mixtures into the first, second and third copper-glass layers 4a, 4b and 5' and the resistor mixture into the resistor 3 as shown in FIG. 2. Then tests were conducted to see what features will come out with change of the amount of copper in the first copper-glass layer 4a which is in contact with the upper side of the resistor 3, and the results are shown in Table 4. The results of tests same as in the first embodiment are also shown in Table 4. As apparent from this table, if the amount of copper in the first copper-glass layer 4a contacting the upper side of the resistor 3 is greater than the amount of copper in the second copper-glass layer 4b on said first copper-glass layer 4a and the softening point of glass to be added to the main resistor mixture containing tin oxide is lower than 600°C and also if the amount of glass added to said main resistor mixture is within the range of 25 to 62 volume percent of said mixture, the variations in resistivity of the obtained spark plugs are as equally limited as the resistor built-in spark plugs obtained in the first embodiment, and also change of resistivity after the spark discharge test, heating test and engine endurance test is very small. Usually, the copper-glass layers contacting the center electrode 6 and middle stem 2 are required to have the following properties: electroconductivity, pressure resistance and air-tightness so as to withstand gas pressure from the internal combustion engine and to maintain airtightness, and ability to ensure mechanical solidity of the center electrode 6 and middle stem 2 and dispersion of heat. It is known that, for providing such properties, each copper-glass layer must contain copper in an amount of 10 to 35 volume percent of glass. In this embodiment of the present invention, the copper-glass layer between the resistor 3 and the middle stem 2 is divided into two sub-layers, and it is essential that the amount of copper in the first copper-glass layer 4a contacting the upper side of the resistor is greater than the amount of copper in the second layer 4b contacting the middle stem 2, so that the rate of copper to glass must be higher than the above-said range of 10 to 35 volume percent. It was, however, found that there is a certain threshold limit for obtaining any significant result, that is, it was found that although not clearly shown in Table 4, the above-said effect can not be produced unless copper is blended in an amount of more than 30 volume percent of glass. Therefore, if copper is blended in the second copper-glass layer 4b in an amount of 10 volume percent of glass in said layer 4b, it suffices to blend copper in the first copper-glass layer 4a in an amount of more than 30 volume percent of glass in said layer 4a. However, if the amount of copper blended in the second copper-glass layer 4b on the side of the middle stem 2 is 30

volume percent of glass in said layer 4b, it is obviously quite meaningless to blend copper in the first copper-glass layer 4a in an amount of 30 volume percent of glass in said layer 4a. Therefore, in case the amount of copper in the second copper-glass layer 4b on the middle stem side is greater than 10 volume percent but smaller than 30 volume percent of glass in said layer 4b, it will do for the purpose to blend copper in the first layer 4a in an amount of 30 volume percent of glass in said layer 4a, but in case the amount of copper in the second layer 4b is 30 volume percent of glass in said layer 4b, the amount of copper blended in the first layer 4a contacting the upper side of the resistor 3 must be greater than 30 volume percent of glass in said layer 4a. Therefore, as apparent from Table 4, if copper is blended in the first layer 4a in an amount of above-said volume percent of glass in said layer 4a, change of resistivity after the spark discharge test, heating test and engine endurance test is extremely limited, and further, even when using glass with high coefficient of expansion (such as glass of specimen No. 14 where  $\alpha = 14.0 \times 10^{-6}/^{\circ}\text{C}$ ), the percent defective, or the rate of defective articles whose resistivities are outside the range of  $5 \text{ K}\Omega \pm 30\%$  (3.5 to 6.5  $\text{K}\Omega$ ) is 11 percent, that is, 11 out of every 100 articles manufactured. This is a marked improvement as compared with 45 percent defectives resulting from use of glass of specimen No. 14 as shown in Table 2. The number of experiments in this second embodiment is small as compared with that in the first embodiment, but this is due to the fact that the second embodiment was practiced on the basis of the first embodiment. Therefore, the softening temperature of glass to be added to the main resistor mixture containing tin oxide, the amount of glass to be added, and the softening temperature of glass in the first, second and third copper-glass layers are all same as those in the first embodiment.

If glass with high coefficient of expansion is used as glass component of the resistor 3, the difference of thermal expansion in the resistor 3 is further added to the difference of thermal expansion between the insulator 1 and the middle stem 2, so that thermal stress develops in the middle stem 2 in the cooling step after manufacture of the spark plug to pull the copper-glass layer which contacts the middle stem 2, with the result that cracks are produced in said copper-glass layer or in the juncture of said layer and the resistor, and this causes variations in resistivity such as above-said. Such problem, however, is eliminated according to this second embodiment of the invention for the following reasons. That is, if the amount of copper contained in the first copper-glass layer 4a contacting the resistor 3 is increased as compared with the amount of copper in the second layer 4b contacting the stem 2, the amount of glass in said layer 4a is naturally decreased to invite reduction of mutual bonding strength of the copper particles. Consequently, cracks develop in the first copper-glass layer 4a containing greater amount of copper owing to tensile force produced by thermal expansion of the middle stem 2, and such cracks mitigate said tensile force to an extent where such force can no longer exert any influence to the resistor 3. Therefore, even if cracks are produced in the first copper-glass layer 4a where copper is abundant, copper, for its excellent malleability, extends out in conformity to such cracks to bridge the cracked portion, thus securing current passage between the stem 2 and the center electrode 6.

Now, the third embodiment of the present invention is described. There were prepared fine particles of glass (all passing 200-mesh screen) of specimen Nos. 4, 5, 19 and 20 of Table 1, and a powdery main resistor mixture containing tin oxide added with 3 wt percent of antimony oxide and 10 wt percent of tantalum oxide, then burned at 1200°C and then pulverized. Each of said glass specimens and the pulverized main resistor mixture containing tin oxide were collected in suitable measured amounts, and then they were well mixed up in a ball mill to obtain resistor mixture. There were also prepared copper powder (wholly passing 200-mesh screen) and pulverized glass of specimen Nos. 1 and 3 of Table 1, and then said copper powder and pulverized glass of each specimen were mixed at the respectively predetermined rates to obtain mixture powders. Then, one of said mixture powders was charged onto the center electrode 6 in the hole 1a in the insulator 1, then another mixture powder different in amount of copper from the first-said mixture powder was charged thereon, and then said resistor mixture was charged on said another mixture powder, this being followed by additional charge thereon of still another mixture powder different in copper amount from the previous mixture powders and final charge thereon of the first-said mixture powder, as shown in FIG. 3. Thereafter, the middle stem 2 was inserted topwise into said hole 1a and subjected to hot press, thereby forming said respective mixture powders into the first, second, third

and fourth copper-glass layers 4a, 4b, 5a and 5b, and the resistor mixture into the resistor 3 as shown in FIG. 3. Then experiments were carried out to see how the effects vary with change of the amount of copper in the 5 first and third copper-glass layers 4a and 5a contacting the upper and lower sides of the resistor 3. The results of these experiments are given in Table 4 along with the results of the tests same as conducted in the first embodiment. As apparent from this table, the above-dis-10 cussed third embodiment produces as excellent results as in the first and second embodiments. The results after the spark discharge test, heating test and engine endurance test are also satisfactory. In this third embodiment, too, it is essential that the amount of copper blended in the first and third copper-glass layers 4a and 5a is within the perfectly same range of volume 15 percent (of glass in said respective layers 4a and 5a) as in the second embodiment. The number of experiments in this third embodiment is small as compared with that 20 in the first embodiment, but this is due to the fact that the third embodiment was practiced on the basis of the first and second embodiments. Therefore, the softening temperature of glass to be added to the main resistor mixture containing tin oxide, the amounts of glass to be 25 added, and the softening temperature of glass in the first, second, third and fourth copper-glass layers 4a, 4b, 5a and 5b are all completely same as those in the first embodiment.

Table 1

| Glass Specimen No. | Components and Properties of Various Types (Specimens) of Glass Used |                  |     |     |                               |                                |                  |      |                  |     | Thermal expansion ( $\times 10^{-6}/^{\circ}\text{C}$ ) | Softening temperature (°C) |      |
|--------------------|----------------------------------------------------------------------|------------------|-----|-----|-------------------------------|--------------------------------|------------------|------|------------------|-----|---------------------------------------------------------|----------------------------|------|
|                    | Na <sub>2</sub> O                                                    | K <sub>2</sub> O | CaO | MgO | B <sub>2</sub> O <sub>3</sub> | Al <sub>2</sub> O <sub>3</sub> | SiO <sub>2</sub> | PbO  | TiO <sub>2</sub> | ZnO | P <sub>2</sub> O <sub>5</sub>                           |                            |      |
| 1                  | 7                                                                    |                  |     |     | 2.3                           | 16                             | 64               |      |                  |     |                                                         | 4.3                        | 590  |
| 2                  | 6                                                                    | 2.5              | 3.5 |     | 13                            | 16                             | 59               |      |                  |     |                                                         | 7.4                        | 570  |
| 3                  | 9                                                                    |                  |     |     |                               | 5                              | 72               |      |                  |     |                                                         | 6.0                        | 760  |
| 4                  |                                                                      |                  |     |     | 17.3                          |                                |                  | 82.7 |                  |     |                                                         | 11.3                       | 360  |
| 5                  |                                                                      |                  |     |     | 11                            | 11                             | 3                | 75   |                  |     |                                                         | 8.3                        | 440  |
| 6                  |                                                                      |                  |     |     | 30                            |                                |                  | 70   |                  |     |                                                         | 8.6                        | 448  |
| 7                  |                                                                      |                  |     |     | 31.7                          |                                |                  | 68.3 |                  |     |                                                         | 8.6                        | 451  |
| 8                  |                                                                      |                  |     |     | 34.9                          |                                |                  | 65.1 |                  |     |                                                         | 7.9                        | 493  |
| 9                  |                                                                      |                  |     |     | 44.6                          |                                |                  | 55.4 |                  |     |                                                         | 6.3                        | 540  |
| 10                 |                                                                      |                  |     |     | 75                            |                                |                  | 25.0 |                  |     |                                                         | 5.7                        | 705  |
| 11                 | 9.5                                                                  |                  |     |     | 39.2                          |                                | 43.2             |      | 8.1              |     |                                                         | 6.6                        | 730  |
| 12                 | 28.0                                                                 |                  |     |     | 41.9                          |                                | 18.1             |      | 12.0             |     |                                                         | 13.2                       | 580  |
| 13                 | 18.4                                                                 |                  |     |     | 3.8                           |                                | 34.2             |      | 33.6             |     |                                                         | 10.3                       | 700  |
| 14                 | 39                                                                   |                  |     |     | 32                            |                                | 14               |      | 15               |     |                                                         | 14.0                       | 500  |
| 15                 |                                                                      |                  |     |     | V <sub>2</sub> O <sub>5</sub> | 30                             |                  |      | 60               |     |                                                         | 5.2                        | 440  |
| 16                 |                                                                      |                  |     |     | 10                            |                                |                  |      | 50               |     |                                                         | 5.1                        | 480  |
| 17                 |                                                                      |                  |     |     | V <sub>2</sub> O <sub>5</sub> | 20                             |                  |      |                  |     |                                                         | 5.2                        | 576  |
| 18                 |                                                                      |                  |     |     | 30                            |                                |                  |      |                  |     |                                                         | 4.6                        | 620  |
| 19                 | 14                                                                   |                  |     |     | 10                            | 50                             |                  |      | 40               |     |                                                         | 33.5                       | 12.4 |
| 20                 |                                                                      |                  |     |     | 45                            |                                |                  |      | 55               |     |                                                         | 70                         | 360  |
| 21                 |                                                                      |                  |     |     | 10                            | 4                              | 12               |      |                  |     |                                                         | 40                         | 400  |
| 22                 |                                                                      |                  |     |     | 10                            | 10                             | 30               |      |                  |     |                                                         | 21.6                       | 530  |
|                    |                                                                      |                  |     |     | 13.6                          | 38.1                           | 21.7             |      |                  |     |                                                         |                            | 700  |

Table 2-1

| Specimen No. in Copper-glass Layers of electrode | Resistor portion              |                                    |                                                                                            |                                                                                                                    | Results                                                                         |                                                              |                                                                       |  |  |  |
|--------------------------------------------------|-------------------------------|------------------------------------|--------------------------------------------------------------------------------------------|--------------------------------------------------------------------------------------------------------------------|---------------------------------------------------------------------------------|--------------------------------------------------------------|-----------------------------------------------------------------------|--|--|--|
|                                                  | Glass Specimen No. of Table 1 | Amount of glass blended (volume %) | Average resistivity (KΩ) of every 100 pieces of resistor built-in spark plugs manufactured | Fraction defective (%) (Rate of the detective articles whose resistivities are outside the range of 3.5 to 6.5 KΩ) | Rate of change of average resistivity after one-minute spark discharge test (%) | Rate of change of average resistivity after heating test (%) | Rate of change of average resistivity after engine endurance test (%) |  |  |  |
| 1                                                | 1                             | 50                                 | 6                                                                                          | 50                                                                                                                 | 6                                                                               | 8                                                            | 7                                                                     |  |  |  |
| 1                                                | 2                             | 50                                 | 6                                                                                          | 25                                                                                                                 | 5                                                                               | 4                                                            | 5                                                                     |  |  |  |
| 1                                                | 2                             | 57                                 | 6.3                                                                                        | 27                                                                                                                 | 5                                                                               | 5                                                            | 5                                                                     |  |  |  |
| 1                                                | 2                             | 64                                 | 6.5                                                                                        | 60                                                                                                                 | 20                                                                              | 15                                                           | 10                                                                    |  |  |  |
| 1                                                | 4                             | 50                                 | 5.8                                                                                        | 25                                                                                                                 | 5                                                                               | 4                                                            | 20                                                                    |  |  |  |
| 1                                                | 5                             | 50                                 | 5.1                                                                                        | 5                                                                                                                  | 5                                                                               | 3                                                            | 5                                                                     |  |  |  |

Table 2-1-continued

| Specimen No. in Copper-glass Layers of electrode | Resistor portion        |       |                                    | Results                                                                                    |                                                                                                                    |                                                                                 |                                                              |
|--------------------------------------------------|-------------------------|-------|------------------------------------|--------------------------------------------------------------------------------------------|--------------------------------------------------------------------------------------------------------------------|---------------------------------------------------------------------------------|--------------------------------------------------------------|
|                                                  | Specimen No. of Table 1 | Glass | Amount of glass blended (volume %) | Average resistivity (KΩ) of every 100 pieces of resistor built-in spark plugs manufactured | Fraction defective (%) (Rate of the defective articles whose resistivities are outside the range of 3.5 to 6.5 KΩ) | Rate of change of average resistivity after one-minute spark discharge test (%) | Rate of change of average resistivity after heating test (%) |
| 1                                                | 5                       | 40    | 5.0                                | 6                                                                                          | 5                                                                                                                  | 3                                                                               | 5                                                            |
| 1                                                | 5                       | 27    | 5.3                                | 7                                                                                          | 5                                                                                                                  | 10                                                                              | 3                                                            |
| 1                                                | 5                       | 57    | 5.7                                | 5                                                                                          | 5                                                                                                                  | 4                                                                               | 5                                                            |
| 1                                                | 5                       | 64    | 6.7                                | 50                                                                                         | 15                                                                                                                 | 10                                                                              | 8                                                            |
| 1                                                | 6                       | 47    | 5.1                                | 4                                                                                          | 5                                                                                                                  | 5                                                                               | 5                                                            |
| 1                                                | 7                       | 40    | 5.0                                | 5                                                                                          | 4                                                                                                                  | 5                                                                               | 6                                                            |
| 1                                                | 8                       | 55    | 5.3                                | 5                                                                                          | 5                                                                                                                  | 4                                                                               | 7                                                            |
| 1                                                | 9                       | 50    | 5.1                                | 5                                                                                          | 5                                                                                                                  | 5                                                                               | 5                                                            |
| 1                                                | 9                       | 64    | 6.8                                | 52                                                                                         | 15                                                                                                                 | 11                                                                              | 7                                                            |
| 1                                                | 10                      | 47    | 6.3                                | 60                                                                                         | 5                                                                                                                  | 20                                                                              | 21                                                           |
| 1                                                | 11                      | 50    | 6.5                                | 70                                                                                         | 7                                                                                                                  | 20                                                                              | 21                                                           |
| 1                                                | 12                      | 50    | 5.8                                | 65                                                                                         | 5                                                                                                                  | 5                                                                               | 6                                                            |
| 1                                                | 13                      | 47    | 6.5                                | 60                                                                                         | 5                                                                                                                  | 21                                                                              | 20                                                           |
| 1                                                | 14                      | 47    | 5.9                                | 45                                                                                         | 5                                                                                                                  | 5                                                                               | 5                                                            |
| 3                                                | 1                       | 50    | 6.0                                | 8                                                                                          | 6                                                                                                                  | 7                                                                               | 7                                                            |
| 11                                               | 2                       | 50    | 6.1                                | 7                                                                                          | 5                                                                                                                  | 5                                                                               | 4                                                            |
| 3                                                | 10                      | 45    | 6.2                                | 20                                                                                         | 5                                                                                                                  | 21                                                                              | 22                                                           |
| 3                                                | 11                      | 50    | 6.2                                | 28                                                                                         | 7                                                                                                                  | 20                                                                              | 21                                                           |
| 3                                                | 13                      | 50    | 6.4                                | 30                                                                                         | 6                                                                                                                  | 22                                                                              | 20                                                           |
| 3                                                | 18                      | 50    | 6.1                                | 25                                                                                         | 7                                                                                                                  | 17                                                                              | 19                                                           |
| 3                                                | 22                      | 45    | 6.1                                | 23                                                                                         | 6                                                                                                                  | 21                                                                              | 21                                                           |
| 1                                                | 3                       | 45    | 6.5                                | 70                                                                                         | 7                                                                                                                  | 25                                                                              | 25                                                           |

Table 2-2

| Specimen No. in Copper-glass Layers of electrode | Resistor portion        |       |                                    | Results                                                                                    |                                                                                                                    |                                                                                 |                                                              |
|--------------------------------------------------|-------------------------|-------|------------------------------------|--------------------------------------------------------------------------------------------|--------------------------------------------------------------------------------------------------------------------|---------------------------------------------------------------------------------|--------------------------------------------------------------|
|                                                  | Specimen No. of Table 1 | Glass | Amount of glass blended (volume %) | Average Resistivity (KΩ) of every 100 pieces of resistor built-in spark plugs manufactured | Fraction defective (%) (Rate of the defective articles whose resistivities are outside the range of 3.5 to 6.5 KΩ) | Rate of change of average resistivity after one-minute spark discharge test (%) | Rate of change of average resistivity after heating test (%) |
| 1                                                | 15                      | 27    | 5.4                                | 6                                                                                          | 5                                                                                                                  | 10                                                                              | 8                                                            |
| 1                                                | 15                      | 33    | 5.0                                | 5                                                                                          | 5                                                                                                                  | 4                                                                               | 5                                                            |
| 1                                                | 15                      | 55    | 5.9                                | 5                                                                                          | 5                                                                                                                  | 5                                                                               | 7                                                            |
| 1                                                | 16                      | 64    | 7.0                                | 55                                                                                         | 15                                                                                                                 | 12                                                                              | 8                                                            |
| 1                                                | 16                      | 50    | 4.8                                | 5                                                                                          | 4                                                                                                                  | 5                                                                               | 4                                                            |
| 1                                                | 17                      | 50    | 6.0                                | 35                                                                                         | 7                                                                                                                  | 5                                                                               | 7                                                            |
| 1                                                | 13                      | 50    | 6.2                                | 55                                                                                         | 6                                                                                                                  | 19                                                                              | 20                                                           |
| 1                                                | 18                      | 38    | 4.5                                | 50                                                                                         | 5                                                                                                                  | 20                                                                              | 20                                                           |
| 1                                                | 19                      | 50    | 5.8                                | 45                                                                                         | 6                                                                                                                  | 5                                                                               | 7                                                            |
| 1                                                | 20                      | 50    | 6.0                                | 50                                                                                         | 7                                                                                                                  | 5                                                                               | 6                                                            |
| 1                                                | 21                      | 50    | 4.7                                | 5                                                                                          | 5                                                                                                                  | 4                                                                               | 4                                                            |
| 1                                                | 22                      | 42    | 6.4                                | 55                                                                                         | 7                                                                                                                  | 23                                                                              | 24                                                           |
| 2                                                | 5                       | 50    | 5.0                                | 5                                                                                          | 5                                                                                                                  | 4                                                                               | 6                                                            |
| 3                                                | 5                       | 57    | 5.5                                | 4                                                                                          | 5                                                                                                                  | 4                                                                               | 6                                                            |
| 3                                                | 9                       | 50    | 5.2                                | 5                                                                                          | 4                                                                                                                  | 5                                                                               | 5                                                            |
| 3                                                | 16                      | 38    | 5.0                                | 5                                                                                          | 6                                                                                                                  | 5                                                                               | 7                                                            |
| 1                                                | 5                       | 20    | 4.5                                | 10                                                                                         | 6                                                                                                                  | 5                                                                               | 8                                                            |
| 1                                                | 5                       | 15    | 4.0                                | 10                                                                                         | 8                                                                                                                  | 5                                                                               | 8                                                            |
| 1                                                | 5                       | 12    | 4.0                                | 15                                                                                         | 10                                                                                                                 | 14                                                                              | 10                                                           |
| 1                                                | 5                       | 10    | 3.8                                | 30                                                                                         | 50                                                                                                                 | 16                                                                              | 12                                                           |
| 9                                                | 21                      | 50    | 5.2                                | 45                                                                                         | 5                                                                                                                  | 5                                                                               | 5                                                            |
| 2                                                | 1                       | 50    | 6.3                                | 50                                                                                         | 7                                                                                                                  | 9                                                                               | 6                                                            |
| 18                                               | 1                       | 50    | 6.0                                | 11                                                                                         | 7                                                                                                                  | 8                                                                               | 6                                                            |
| 9                                                | 1                       | 50    | 6.3                                | 55                                                                                         | 8                                                                                                                  | 7                                                                               | 8                                                            |
| 2                                                | 2                       | 50    | 6.1                                | 50                                                                                         | 5                                                                                                                  | 5                                                                               | 5                                                            |
| 22                                               | 2                       | 50    | 6.0                                | 10                                                                                         | 5                                                                                                                  | 5                                                                               | 6                                                            |
| 21                                               | 9                       | 50    | 5.1                                | 48                                                                                         | 5                                                                                                                  | 6                                                                               | 7                                                            |
| 2                                                | 9                       | 45    | 5.2                                | 10                                                                                         | 5                                                                                                                  | 4                                                                               | 6                                                            |
| 3                                                | 12                      | 38    | 5.3                                | 45                                                                                         | 5                                                                                                                  | 5                                                                               | 5                                                            |
| 2                                                | 17                      | 50    | 6.8                                | 60                                                                                         | 7                                                                                                                  | 6                                                                               | 7                                                            |
| 3                                                | 17                      | 50    | 6.2                                | 10                                                                                         | 6                                                                                                                  | 5                                                                               | 5                                                            |
| 9                                                | 21                      | 50    | 5.0                                | 38                                                                                         | 6                                                                                                                  | 5                                                                               | 5                                                            |
| 2                                                | 21                      | 50    | 4.8                                | 6                                                                                          | 6                                                                                                                  | 5                                                                               | 6                                                            |

Table 2-3

| Specimen No. in Copper-glass Layers of electrode | Resistor portion              |                                    |                                                                                            | Results                                                                                                            |                                                                                 |                                                              |                                                                       |
|--------------------------------------------------|-------------------------------|------------------------------------|--------------------------------------------------------------------------------------------|--------------------------------------------------------------------------------------------------------------------|---------------------------------------------------------------------------------|--------------------------------------------------------------|-----------------------------------------------------------------------|
|                                                  | Glass Specimen No. of Table 1 | Amount of glass blended (volume %) | Average resistivity (KΩ) of every 100 pieces of resistor built-in spark plugs manufactured | Fraction defective (%) (Rate of the detective articles whose resistivities are outside the range of 3.5 to 6.5 KΩ) | Rate of change of average resistivity after one-minute spark discharge test (%) | Rate of change of average resistivity after heating test (%) | Rate of change of average resistivity after engine endurance test (%) |
| 1                                                | 5                             | 43                                 | 4.5                                                                                        | 10                                                                                                                 | 5                                                                               | 5                                                            | 5                                                                     |
| 1                                                | "                             | 55                                 | 4.8                                                                                        | 8                                                                                                                  | 6                                                                               | 4                                                            | 5                                                                     |
| 1                                                | "                             | 62                                 | 5.2                                                                                        | 12                                                                                                                 | 8                                                                               | 5                                                            | 5                                                                     |
| 1                                                | "                             | 20                                 | 3.5                                                                                        | 80                                                                                                                 | 8                                                                               | 25                                                           | 15                                                                    |
| 1                                                | "                             | 38                                 | 4.3                                                                                        | 8                                                                                                                  | 5                                                                               | 4                                                            | 5                                                                     |
| 1                                                | "                             | 49                                 | 4.5                                                                                        | 5                                                                                                                  | 5                                                                               | 3                                                            | 8                                                                     |
| 1                                                | "                             | 57                                 | 5.2                                                                                        | 15                                                                                                                 | 4                                                                               | 6                                                            | 7                                                                     |
| 1                                                | "                             | 63                                 | 6.8                                                                                        | 63                                                                                                                 | 8                                                                               | 20                                                           | 10                                                                    |
| 1                                                | "                             | 33                                 | 4.0                                                                                        | 15                                                                                                                 | 7                                                                               | 7                                                            | 5                                                                     |
| 1                                                | "                             | 44                                 | 4.5                                                                                        | 10                                                                                                                 | 6                                                                               | 6                                                            | 5                                                                     |
| 1                                                | "                             | 52                                 | 5.6                                                                                        | 10                                                                                                                 | 7                                                                               | 5                                                            | 8                                                                     |
| 1                                                | "                             | 14                                 | 2.2                                                                                        | 90                                                                                                                 | 5                                                                               | 35                                                           | 20                                                                    |
| 1                                                | "                             | 40                                 | 4.5                                                                                        | 12                                                                                                                 | 8                                                                               | 5                                                            | 7                                                                     |
| 1                                                | "                             | 48                                 | 5.6                                                                                        | 10                                                                                                                 | 7                                                                               | 8                                                            | 8                                                                     |
| 1                                                | "                             | 12                                 | 2.0                                                                                        | 98                                                                                                                 | 10                                                                              | 35                                                           | 25                                                                    |
| 1                                                | "                             | 25                                 | 5.3                                                                                        | 15                                                                                                                 | 5                                                                               | 10                                                           | 8                                                                     |

Table 3

| Specimen<br>No. of<br>glass<br>in the<br>copper-<br>glass<br>layers | Filler<br>Material | Resistor<br>portion                            |                                        |                                                                                                                            | Results                                                                                                                                     |                                                                                                                 |                                                                                     |                                                                                              |    |
|---------------------------------------------------------------------|--------------------|------------------------------------------------|----------------------------------------|----------------------------------------------------------------------------------------------------------------------------|---------------------------------------------------------------------------------------------------------------------------------------------|-----------------------------------------------------------------------------------------------------------------|-------------------------------------------------------------------------------------|----------------------------------------------------------------------------------------------|----|
|                                                                     |                    | Glass<br>speci-<br>men<br>No. of<br>Table<br>1 | Amount<br>of<br>glass<br>(volume<br>%) | Average<br>resist-<br>ivity (KΩ)<br>of every<br>100 pieces<br>of resistor<br>built-<br>in spark<br>plugs manu-<br>factured | Fraction<br>defective<br>(%) (Rate of<br>defective<br>articles<br>whose resis-<br>tivities are<br>outside the<br>range of 3.5<br>to 6.5 KΩ) | Rate of<br>change of<br>average<br>resist-<br>ivity<br>after one-<br>minute<br>spark dis-<br>charge<br>test (%) | Rate of<br>change of<br>average<br>resist-<br>ivity<br>after<br>heating<br>test (%) | Rate of<br>change of<br>average<br>resist-<br>ivity after<br>engine<br>endurance<br>test (%) |    |
| 1                                                                   | F.Q.               | 20                                             | 5                                      | 47                                                                                                                         | 5.5                                                                                                                                         | 5                                                                                                               | 5                                                                                   | 4                                                                                            | 5  |
| 1                                                                   | ZrO <sub>2</sub>   | "                                              | "                                      | 48                                                                                                                         | 5.4                                                                                                                                         | 5                                                                                                               | 5                                                                                   | 4                                                                                            | 5  |
| 1                                                                   | ZrO <sub>2</sub>   | "                                              | "                                      | 48                                                                                                                         | 5.5                                                                                                                                         | 5                                                                                                               | 6                                                                                   | 5                                                                                            | 4  |
|                                                                     | SiO <sub>2</sub>   | "                                              | "                                      | 8                                                                                                                          | 35                                                                                                                                          | 5.2                                                                                                             | 5                                                                                   | 5                                                                                            | 7  |
| 1                                                                   | "                  | "                                              | "                                      | 53                                                                                                                         | 5.7                                                                                                                                         | 8                                                                                                               | 5                                                                                   | 4                                                                                            | 6  |
| 1                                                                   | "                  | "                                              | "                                      | 63                                                                                                                         | 7.5                                                                                                                                         | 80                                                                                                              | 20                                                                                  | 12                                                                                           | 10 |
| 1                                                                   | F.Q.               | "                                              | 4                                      | 47                                                                                                                         | 5.6                                                                                                                                         | 15                                                                                                              | 5                                                                                   | 5                                                                                            | 8  |
| 3                                                                   | "                  | "                                              | 12                                     | 47                                                                                                                         | 5.7                                                                                                                                         | 18                                                                                                              | 5                                                                                   | 5                                                                                            | 5  |
| 1                                                                   | F.Q.               | 20                                             | 14                                     | 47                                                                                                                         | 5.6                                                                                                                                         | 20                                                                                                              | 5                                                                                   | 5                                                                                            | 6  |
| 1                                                                   | "                  | "                                              | 14                                     | 23                                                                                                                         | 5.8                                                                                                                                         | 8                                                                                                               | 5                                                                                   | 20                                                                                           | 7  |
| 1                                                                   | "                  | "                                              | 20                                     | 41                                                                                                                         | 5.1                                                                                                                                         | 12                                                                                                              | 5                                                                                   | 5                                                                                            | 6  |
| 1                                                                   | "                  | 30                                             | 20                                     | 40                                                                                                                         | 8.0                                                                                                                                         | (98)                                                                                                            | 5                                                                                   | 5                                                                                            | 7  |
| 1                                                                   | "                  | 20                                             | 5                                      | 27                                                                                                                         | 5.6                                                                                                                                         | 7                                                                                                               | 5                                                                                   | 10                                                                                           | 8  |

(Note)

(Note)  
F.Q. = quartz glass

$\text{ZrO}_3$  = zircon

$\text{ZrO}_2 \cdot \text{SiO}_2 = \text{zircon}$

Table 4

| Copper-glass Layer portion of electrode |                                    |                             |                                    |                                 |                                    |                              |                                    |                               |    | Resistor                          |
|-----------------------------------------|------------------------------------|-----------------------------|------------------------------------|---------------------------------|------------------------------------|------------------------------|------------------------------------|-------------------------------|----|-----------------------------------|
| Second copper-glass layer 4b            |                                    | First copper-glass layer 4a |                                    | Third copper-glass layer 5', 5a |                                    | Fourth copper-glass layer 5b |                                    | Glass specimen No. of Table 1 |    | Amount of glass blended (volume%) |
| Glass specimen No.                      | Amount of copper blended (volume%) | Glass specimen No.          | Amount of copper blended (volume%) | Glass specimen No.              | Amount of copper blended (volume%) | Glass specimen No.           | Amount of copper blended (volume%) | Glass specimen No. of Table 1 |    |                                   |
| Second embodiment                       | 1                                  | 23                          | 1                                  | 41                              | —                                  | —                            | 1                                  | 23                            | 5  | 50                                |
|                                         | 1                                  | 10                          | 1                                  | 41                              | —                                  | —                            | 1                                  | 10                            | 5  | 50                                |
|                                         | 1                                  | 23                          | 2                                  | 53                              | —                                  | —                            | 1                                  | 23                            | 5  | 50                                |
|                                         | 1                                  | 23                          | 2                                  | 30                              | —                                  | —                            | 1                                  | 23                            | 9  | 50                                |
|                                         | 1                                  | 23                          | 1                                  | 53                              | —                                  | —                            | 1                                  | 23                            | 4  | 50                                |
|                                         | 1                                  | 23                          | 1                                  | 30                              | —                                  | —                            | 1                                  | 23                            | 4  | 50                                |
|                                         | 2                                  | 23                          | 2                                  | 41                              | —                                  | —                            | 1                                  | 23                            | 14 | 50                                |
| Third embodiment                        | 3                                  | 23                          | 3                                  | 53                              | 3                                  | 53                           | 3                                  | 23                            | 20 | 50                                |
|                                         | 3                                  | 20                          | 3                                  | 30                              | 3                                  | 30                           | 3                                  | 20                            | 19 | 50                                |
|                                         | 1                                  | 10                          | 1                                  | 53                              | 1                                  | 53                           | 1                                  | 10                            | 4  | 50                                |
|                                         | 1                                  | 30                          | 1                                  | 53                              | 1                                  | 53                           | 1                                  | 30                            | 4  | 50                                |
|                                         | 1                                  | 23                          | 1                                  | 53                              | 1                                  | 53                           | 1                                  | 23                            | 4  | 50                                |
|                                         | 1                                  | 23                          | 1                                  | 74                              | 1                                  | 74                           | 1                                  | 23                            | 5  | 50                                |

Table 4-continued

| Average resistivity (KΩ) of every 100 pieces of resistor built-in spark plugs manufactured | Fraction defective (%) (Rate of defective articles whose resistivities are outside the range of 3.5 to 6.5 KΩ) | Results<br>Rate of change of average resistivity after one-minute spark discharge test (%) | Rate of change of average resistivity after heating test (%) | Rate of change of average resistivity after engine endurance test (%) |
|--------------------------------------------------------------------------------------------|----------------------------------------------------------------------------------------------------------------|--------------------------------------------------------------------------------------------|--------------------------------------------------------------|-----------------------------------------------------------------------|
| 5.0                                                                                        | 5                                                                                                              | 5                                                                                          | 3                                                            | 5                                                                     |
| 5.1                                                                                        | 5                                                                                                              | 5                                                                                          | 4                                                            | 5                                                                     |
| 5.1                                                                                        | 5                                                                                                              | 5                                                                                          | 3                                                            | 5                                                                     |
| 5.0                                                                                        | 5                                                                                                              | 4                                                                                          | 4                                                            | 5                                                                     |
| 5.4                                                                                        | 12                                                                                                             | 5                                                                                          | 5                                                            | 7                                                                     |
| 5.3                                                                                        | 12                                                                                                             | 5                                                                                          | 5                                                            | 6                                                                     |
| 5.5                                                                                        | 11                                                                                                             | 5                                                                                          | 4                                                            | 6                                                                     |
| 5.7                                                                                        | 15                                                                                                             | 6                                                                                          | 6                                                            | 7                                                                     |
| 5.5                                                                                        | 12                                                                                                             | 5                                                                                          | 5                                                            | 6                                                                     |
| 5.3                                                                                        | 11                                                                                                             | 5                                                                                          | 5                                                            | 6                                                                     |
| 5.3                                                                                        | 11                                                                                                             | 5                                                                                          | 5                                                            | 6                                                                     |
| 5.4                                                                                        | 5                                                                                                              | 5                                                                                          | 5                                                            | 5                                                                     |
| 5.0                                                                                        | 5                                                                                                              | 5                                                                                          | 3                                                            | 5                                                                     |

The volume percent of glass blended into the main resistor mixture containing tin oxide was found from the results of our experiments and determined to take certain specified times of void volume of said mixture.

In each of the foregoing embodiments of the invention, there have been obtained the resistor built-in spark plugs having resistivity of  $5 \text{ K}\Omega \pm 1.5 \text{ K}\Omega$  as apparent from the tables given for the respective embodiments, but it is possible to obtain the spark plugs having resistivities of other ranges, for example  $10 \text{ K}\Omega \pm 3 \text{ K}\Omega$  and  $15 \text{ K}\Omega \pm 4.5 \text{ K}\Omega$ , by suitably changing the rate of tin oxide contained in the resistor and the amounts of additives such as tantalum oxide. In these cases, the amount of glass added to the main resistor mixture containing tin oxide and the softening point of such glass are of course within the above-defined ranges.

What is claimed is

1. A resistor built-in spark plug comprising an insulator formed with an axially extending inner hole, a stem fitted in the upper part of said hole in said insulator, a center electrode fitted in the lower part of said hole, a resistor disposed in the central part of said hole, and copper-glass electrode layers disposed between said resistor and said stem and between said resistor and said center electrode, said resistor being made by firing and solidifying powder of resistor mixture consisting of 75 to 38 volume percent of main resistor component containing tin oxide and 25 to 62 volume percent of glass powder with softening temperature of  $300^\circ$  to  $600^\circ\text{C}$ , and said copper-glass electrode layers being made by firing and solidifying a mixture of copper powder and glass powder with the softening temperature of above  $530^\circ\text{C}$  and more than  $30^\circ\text{C}$  higher than the softening point of glass in the resistor portion.

2. A resistor built-in spark plug comprising an insulator formed with an axially extending inner hole, a stem fitted in the upper part of said hole in said insulator, a center electrode fitted in the lower part of said hole, a resistor disposed in the central part of said hole, a first copper-glass electrode layer disposed between said resistor and said stem and in contact with said stem, a second copper-glass electrode layer disposed in contact with said resistor and containing a greater amount of copper than said first copper-glass layer, and a third copper-glass electrode layer disposed between said resistor and said center electrode, said resistor being made by firing and solidifying powder of resistor mix-

ture consisting of 75 to 38 volume percent of main resistor component containing tin oxide and 25 to 62 volume percent of glass powder with softening temperature of  $300^\circ$  to  $600^\circ\text{C}$ , said first and third copper-glass layers being made by firing and solidifying a mixture of 10 to 35 volume percent of copper powder and 90 to 65 volume percent of glass powder with softening temperature of above  $530^\circ\text{C}$  and more than  $30^\circ\text{C}$  higher than the softening point of glass in the resistor portion, and said second copper-glass layer being made by firing and solidifying a mixture of copper powder in an amount of more than 30 volume percent and greater than the amount of copper in said first copper-glass layer and remaining percent of glass powder with softening temperature of above  $530^\circ\text{C}$  and more than  $30^\circ\text{C}$  higher than the softening temperature of glass in the resistor portion.

3. A resistor built-in spark plug comprising an insulator formed with an axially extending inner hole, a stem fitted in the upper part of said hole in said insulator, a center electrode fitted in the lower part of said hole, a resistor disposed in the central part of said hole, a first copper-glass electrode layer disposed between said resistor and said stem and in contact with said stem, a second copper-glass electrode layer disposed in contact with said resistor and containing a greater amount of copper than said first copper-glass layer, a third copper-glass electrode layer disposed between said resistor and said center electrode and in contact with said center electrode, and a fourth copper-glass electrode layer disposed in contact with said resistor and containing a greater amount of copper than said third copper-glass layer, said resistor being made by firing and solidifying powder of resistor mixture consisting of 75 to 38 volume percent of main resistor component containing tin oxide and 25 to 62 volume percent of glass powder with softening temperature of  $300^\circ$  to  $600^\circ\text{C}$ , said first and third copper-glass layers being made by firing and solidifying a mixture of 10 to 35 volume percent of copper powder and 90 to 65 volume percent of glass powder with softening temperature of above  $530^\circ\text{C}$  and more than  $30^\circ\text{C}$  higher than the softening point of glass in the resistor portion, and said second and fourth copper-glass layers being made by firing and solidifying a mixture comprising more than 30 volume percent of copper powder greater in amount than copper in said first and third copper-glass layers and remaining percent of glass powder with softening temperature of

above 530°C and more than 30°C higher than the softening point of glass in the resistor portion.

4. The resistor built-in spark plug according to claim 1, wherein the main component mixture of said resistor contains a filler with extremely high electric resistivity.

5. The resistor built-in spark plug according to claim 4, wherein said filler is one of the following: quartz glass, zirconia and zircon.

6. The resistor built-in spark plug according to claim 2 wherein the main component mixture of said resistor contains a filler with extremely high electric resistivity.

7. The resistor built-in spark plug according to claim 6, wherein said filler is one of the following: quartz glass, zirconia and zircon.

10

15

8. The resistor built-in spark plug according to claim 3, wherein the main component mixture of said resistor contains a filler with extremely high electric resistivity.

9. The resistor built-in spark plug according to claim 8 wherein said filler is one of the following: quartz glass, zirconia and zircon.

10. The resistor built-in spark plug according to claim 1 wherein the glass in the copper-glass layers has a softening point lower than 750°C.

11. The resistor built-in spark plug according to claim 2 wherein the glass in the copper-glass layers has a softening point lower than 750°C.

12. The resistor built-in spark plug according to claim 3 wherein the glass in the copper-glass layers has a softening point lower than 750°C.

\* \* \* \*

20

25

30

35

40

45

50

55

60

65